

March 10, 1953

N. B. EDELMAN

2,630,947

ARTIFICIALLY CURLED FEATHER

Filed Oct. 11, 1948



INVENTOR.  
Norman B. Edelman

W. J. Eccleston,  
ATTORNEY

## UNITED STATES PATENT OFFICE

2,630,947

## ARTIFICIALLY CURLED FEATHER

Norman B. Edelman, Philadelphia, Pa.

Application October 11, 1948, Serial No. 53,946

6 Claims. (Cl. 223—47)

(Granted under Title 35, U. S. Code (1952),  
sec. 266)

## 1

The invention described herein, if patented, may be manufactured and used by or for the Government for governmental purposes without the payment to me of any royalty thereon.

This invention relates to artificially curled feathers. More particularly, the invention is concerned with a method or process for producing a permanent curl in feathers of the land fowl type, or other feathers, which in their natural state are uncurled.

The relative softness and flexibility, or filling power, of duck feathers and duck down, which are naturally curled, is well known. Many attempts to provide substitutes for such naturally curled feathers have heretofore been made. Such attempts have been directed towards utilizing normally straight, or crushed, broken and stripped feathers, with or without a combination of fibers and other materials, in an effort to obtain an equivalency between relative filling power in correlation with the softness of naturally curled feathers, without accomplishing or producing satisfactory results. That is, no substantially permanent equivalent substitute for or simulation of duck feathers and duck down has heretofore been artificially produced from uncurled feathers.

Further, it is generally known that the application of moisture and heat, with or without the use of spaced rollers, will produce only a temporary curl in fibers, feathers, films, and the like, which remain for short periods of time. Similarly, it was discovered that land fowl feathers, and particularly feathers secured from chickens and turkeys, would form a temporary curl when so treated. However, as could be expected, the curvature of the feather stem was not permanent, and this temporary type of curl was not suitable for general usage. However, by the process hereinafter disclosed for securing a thermoset curl, it is believed that the molecular structure of the highly organized feather keratin is disorganized with a reduction of parallelism of the keratin micelles, resulting in a permanent shortening or contraction of the feather stem.

It is, therefore, an object of this invention to provide artificially curled feathers having substantially the filling power and softness characteristics of naturally curled feathers.

It is another object of this invention to provide methods of thermosetting an artificial curl in normally uncurled feathers.

It is a further object of this invention to provide artificially curled feathers of the land fowl type.

## 2

Other objectives and advantages of this invention will be apparent from the following description, when considered in conjunction with the accompanying drawings, wherein:

5 Fig. 1 is a perspective view of a feather mold;

Fig. 2 is a front elevational view showing a heating cabinet for the feather mold;

Fig. 3 illustrates a normally uncurled feather;

10 Fig. 4 illustrates the feather of Fig. 3 artificially curled;

Fig. 5 is a perspective view of a modified feather mold; and

Fig. 6 is a partial front elevational view of a decorative article.

15 Referring to the drawings, a platform 10 supports at its one end a bracket 11, provided with a conventional holding socket 12 and at its opposite end a bracket 13, provided with a drive shaft (not shown), in alignment with the socket portion 12 of bracket 11.

20 Supported between the brackets 11 and 13 is a tubular forming mold or mandrel 14, adapted to be held at one end in socket 12 of bracket 11 and by a conventional chuck 15 at its opposite end. The chuck 15 is mounted upon the drive shaft in the bracket 13, and is adapted to be turned by a conventional pulley 16, also mounted on the drive shaft and driven by belt 17 through suitable motor drive means or the like (not shown).

25 On the tubular forming means 14, secured by chuck 15, between the brackets 11 and 13, a fabric material 18 is spirally wound along its length with placement of numerous uncurled feathers 19 between the forming mandrel 14 and the fabric or the fabric wrappings 18.

30 As illustrated by the Figure 1, the fabric 18 is started at one end of the mandrel 14, with feathers aligned over the flattened surface 18' of the fabric 18 as it is wound upon the forming element 14 in an advancing spiral.

35 As illustrated by the Figure 1, the feathers are secured in a curved position about the forming element 14. As will be evident, one or more wrappings of fabric may be made over the length of the forming member 14, provided the depth of the laminated wrapping is not so great as to prevent passages of steam and heat therethrough.

40 By this means the feathers are secured in a curved position about the forming element 14. As will be evident, one or more wrappings of fabric may be made over the length of the forming member 14, provided the depth of the laminated wrapping is not so great as to prevent passages of steam and heat therethrough.

45 After the feathers have been shaped, by bending in the manner above described, chuck 15 is loosened and the form 14 is placed in the heating cabinet 20. This heating cabinet 20 comprises a closed steaming chamber formed with conventional sides, top and bottom. Within the top portion 20' of cabinet 20 is placed a suitable valve 21, operable, for example, by handle 22 to

control cabinet pressure or to provide an exhaust outlet. As illustrated, the cabinet is constructed with a steam-tight door 23, containing glass window 24, for purposes of examining and determining cabinet and article conditions. Attached to one side wall of the cabinet is a steam pipe 25, having a suitable nozzle and piped inlet within the cabinet 20. The steam flow is adapted to be controlled by conventional valve 26 for introducing dry and live steam into the interior of the cabinet space in the manner hereinafter described.

In operation the steam supplied to cabinet 20 is furnished by suitable dry and live steam apparatus (not shown) at temperatures, pressures and time relationships which are of a predetermined value, between 100° C. and 500° C. at 5 to 30 pounds' pressure per square inch for proportional periods of time varying from 10 minutes to only a few seconds (approximately 4), respectively, irrespective of pressure.

At the base of the cabinet 20 there is provided an air conduit 27, adapted to be supplied by air pump 28 with a forced draft of drying air. This air supply may be from a suitable air-drying and heating furnace, or taken in from the atmosphere, as desired.

As illustrated in Fig. 5, there is provided a preferred type of forming bar 14', having a central open passageway 29, and its body portion provided with numerous perforations 30. This central passageway 29 and perforations 30 permit the passage of steam and heat through the fabric wrappings, and, therefore, to all surfaces of the pre-shaped feathers. With this hollow, perforated molding mandrel 14' fittings are provided on a steam outlet, upon which the tubular mandrel 14' can be mounted to force live steam into the mold to effectively thermo-set a feather stem into a permanent curl.

For a more specific illustration of the method herein disclosed and the product thereby secured, the Fig. 3 is illustrative of a chicken feather having its shaft portion 31 uncurled and in the natural state. This feather is placed, in the manner shown, on the fabric surface 18' and wrapped about the forming mandrel 14, which in this instance is of a 1" diameter size. After being wrapped about the mandrel, the unit is placed in cabinet 20 and subjected for ten seconds to dry steam maintained at a temperature of 120° C. and a pressure of 5 pounds per square inch. Thereafter a suitable quantity of drying air is forced into the chamber 28, which may be allowed to escape therefrom at the outlet valve 24. With this temperature, pressure and time relationship, brittleness of the feather is avoided. For higher pressures and temperatures, it was discovered that similar results are secured by subjecting feathers to a steam treatment for proportionately shorter time intervals. Likewise, with reduced temperatures and high or low pressures, the heating period may be extended for a time period of approximately 10 minutes without making the finished curled feather brittle and, therefore, of no value with respect to its softness characteristic.

As shown in Fig. 4, when the feather of Fig. 3 has passed through the treatment above described and is unwrapped, it has its shaft portion 31 permanently set in a definite curl. It was discovered that, after the heat treatment above provided, with or without the drying action, the feather stem 31 retained its curl.

To illustrate the practical results of curling a

general run of chicken feathers, for example, by subjecting them to a treatment in the nature of that set forth, the actual filling power of such feathers on a comparison basis with duck feathers, based on measurements of pounds per square inch, was found to be within 20 percent, as may be determined by the following table.

TABLE I  
*Comparison of chicken and duck feathers*  
[Based on an average of several tests]

| Material                         | Filling Power at—         |                          |                         |
|----------------------------------|---------------------------|--------------------------|-------------------------|
|                                  | .0005<br>p. s. i.,<br>cm. | 0.02<br>p. s. i.,<br>in. | 0.2<br>p. s. i.,<br>in. |
| Chicken Feathers before curling  | 2.4                       | (3)                      | (3)                     |
| Chicken Feathers after curling   | 6.5                       | .92                      | .70                     |
| Prime Western Grey Duck Feathers | 7.8                       | 1.06                     | .80                     |
| L. I. White Duck Feathers        | 8.3                       | 1.12                     | .83                     |

<sup>1</sup> Height of 20 gm. of feathers fluffed into a glass cylinder 11.5 inches' diameter.

<sup>2</sup> Height of 10 gm. of feathers in a brass cylinder 3.75 inches' diameter.

<sup>3</sup> Not measured.

From the above it will be recognized that at the lowest test pressures used, chicken feathers have been almost trebled in filling power and are approximately (within 20%) equivalent in filling power to the best duck feathers obtainable. Further, by selecting only vane feathers for curling, and curling them by the process herein illustrated, it is possible to substantially equal the filling power of duck feathers. However, as a practical matter, such separation in bulk volumes is very difficult and a comparatively expensive operation.

In making the above test, care must be taken in measuring the filling power of feathers curled by the autoclaving technique, for it is found such feathers immediately after autoclaving are highly charged with static electricity and it takes considerable time (12 hours or more) before this excess charge leaks away. Unless the feathers are measured at humidities of presumably over 50% at room temperatures and at test pressures of not less than .0005 p. s. i., the filling power obtained will be too high because of this static. Recognition is hereby made of the fact that fluffing the feathers causes them, among other reasons, to occupy more volume by virtue of this static electricity produced during fluffing.

On a comparative basis with other known processes, the following table is representative of the improvement herein provided:

TABLE II  
*Increase in filling power by thermo-set feather curling*

| Method                                                  | .0005<br>p. s. i. | .02<br>p. s. i. | .2 to .3<br>p. s. i. |
|---------------------------------------------------------|-------------------|-----------------|----------------------|
| Eugene, Ltd.—Mandrel                                    | Unknown           | 5.2 to 21%      | 5.4%.                |
| Department of Agriculture<br>Warping (without pressure) | do                | 18%             | 5.4%.                |
| 60%                                                     | Unknown           | Unknown         | Unknown.             |
| Thermo-set (as herein provided)                         | 260%              | 64%             | 59%.                 |

In addition to the specific types of forming apparatus indicated above, it has been found that uncurled feathers, which in any case are preferably cleaned before bending, may be bent and held to the curved shape prior to and during the treatment herein provided by any suitable former.

Such formers may be, for example, tubular formers within which the feathers are stuffed and bent thereby into a precurled position, or an apparatus in the nature of a presser having a mandrel of specific curvature, mandrels of other desired shape or curvature, a roller and shoe, or other apparatuses wherein a steaming treatment, as herein provided, is applied during the time of mechanical deformation of the feathers.

In addition to thermo-setting a curl in normally straight feather bodies, it has been discovered that the straight feathers 19 may be carded or garnetted with other fibers, woven, braided, knitted, or the like, with or secured in fabrics, or in fibrous material as yarn or the like, during spinning. Thereafter these materials, as represented by the fabric 32 of Fig. 6, are shaped in the manner and treated by a process such as herein disclosed. There is thus provided a fibrous structure 32, decorated with artificially curled feathers 33, which retain their curl. Further, the feathers may be artificially dyed or stained in a conventional manner, either prior or subsequent to receiving their thermo-set curl, without damage to the feather structure. Obviously dyes or stains affected by the dry steam and heat are not applied prior to the curling treatment.

Having thus disclosed my invention, it will be possible to provide modifications, adaptations and uses not herein described but believed to fall within the scope of the appended claims.

I claim:

1. A method of making a feather-decorated novelty fabric, comprising mounting straight fowl feathers on a fabric base, conjointly and tightly winding said fabric base and said feathers around a mandrel, and admitting heat to said feathers and fabric base while wound around said mandrel until said feathers are permanently thermoset in a curled configuration.

2. The method of imparting a permanent curl to normally uncurled fowl feathers, comprising aligning said feathers on a gas-permeable flexible support in a direction substantially parallel to an edge of said support, conjointly and tightly winding said feathers and support around a mandrel, the shafts of said feathers being in a plane substantially normal to the axis of said mandrel, and applying heat of at least 100° C. to said feathers while thus wound around said mandrel until said feathers are permanently thermoset in a curled configuration.

3. The method of imparting a permanent curl to normally uncurled fowl feathers, comprising aligning said feathers on an elongated strip of gas-permeable flexible material in a direction substantially parallel to the longitudinal axis of said strip, conjointly and tightly winding said feathers and strip in an advancing spiral around a mandrel, and applying heat of at least 100° C. to said feathers while thus wound around said mandrel until said feathers are permanently thermoset in a curled configuration.

4. The method of imparting a permanent curl

to normally uncurled fowl feathers, comprising aligning said feathers on a gas-permeable flexible support in a direction substantially parallel to an edge of said support, conjointly and tightly winding said feathers and support around a hollow mandrel having a large plurality of perforations in its wall, the shafts of said feathers being in a plane substantially normal to the axis of said mandrel, and passing a hot gas having a temperature of at least 100° C. through the interior and through the perforations of said mandrel into contact with said feathers while said feathers are thus wound around said mandrel until said feathers are permanently thermoset in a curled configuration.

5. The method of imparting a permanent curl to normally uncurled fowl feathers, comprising aligning said feathers on an elongated strip of gas-permeable flexible material in a direction substantially parallel to the longitudinal axis of said strip, conjointly and tightly winding said feathers and strip in an advancing spiral around a hollow mandrel having a large plurality of perforations in its wall, and passing a hot gas having a temperature of at least 100° C. through the interior and through the perforations of said mandrel into contact with said feathers while said feathers are thus wound around said mandrel until said feathers are permanently thermoset in a curled configuration.

6. The method of imparting a permanent curl to normally uncurled fowl feathers, comprising aligning said feathers on a gas-permeable flexible support in a direction substantially parallel to an edge of said support, conjointly and tightly winding said feathers and support around a rotating mandrel, the shafts of said feathers being in a plane substantially normal to the axis of said mandrel, arresting the rotation of said mandrel after said support and feathers are wound thereon, and placing said mandrel and the support and feathers which are wound around said mandrel conjointly into a chamber, and heating said chamber to at least 100° C. until said feathers are permanently thermoset in a curled configuration.

NORMAN B. EDELMAN.

#### REFERENCES CITED

The following references are of record in the file of this patent:

#### UNITED STATES PATENTS

| Number    | Name    | Date           |
|-----------|---------|----------------|
| 225,152   | Low     | Mar. 2, 1880   |
| 260,629   | Ward    | July 4, 1882   |
| 1,392,287 | Wever   | Sept. 27, 1921 |
| 2,049,241 | Amkraut | July 28, 1936  |
| 2,074,732 | Nelson  | Mar. 23, 1937  |
| 2,213,316 | Koga    | Sept. 3, 1940  |
| 2,310,642 | Marcy   | Feb. 9, 1943   |

#### FOREIGN PATENTS

| Number  | Country | Date        |
|---------|---------|-------------|
| 26,240  | Austria | May 1, 1906 |
| 541,687 | France  | May 5, 1922 |